# EUROPEAN PATENT SPECIFICATION

(11) **EP 3 135 810 B1**
(45) Date of publication and mention of the grant of the patent: **12.07.2023**
(21) Application number: 16186411.1
(22) Date of filing: 30.08.2016
(51) Int. Cl.: D21H 13/28, D21H 13/00, D21H 13/34

(54) **PAPER MATERIAL COMPRISING CELLULOSE FIBERS AND LEATHER FIBERS AND PROCESS FOR THE PRODUCTION THEREOF**
PAPIERMATERIAL MIT ZELLULOSEFASERN UND LEDERFASERN SOWIE VERFAHREN ZUR HERSTELLUNG DAVON
MATÉRIAU DE PAPIER COMPRENANT DES FIBRES DE CELLULOSE ET DES FIBRES DE CUIR ET SON PROCÉDÉ DE PRODUCTION

(30) Priority: 31.08.2015 IT UB20153307
(43) Date of publication of application: 01.03.2017
(73) Proprietor: Favini S.r.l., 36028 Rossano Veneto, (VI) (IT)
(72) Inventor: MONEGATO, Achille, 31037 LORIA (TV) (IT); STRAGLIOTTO, Flavio, 36027 ROSÀ (VI) (IT); BERNO, Giacomo, 36028 ROSSANO VENETO (VI) (IT); PRUSCINI, Giovanni, 36022 CASSOLA (VI) (IT); DAL BIANCO, Maurizio, 36022 CASSOLA (VI) (IT)
(74) Representative: Marturano, Pasqualino

(56) References cited:
- GB-A- 2 045 829
- US-A- 1 211 837
- US-A- 1 269 905
- US-A- 2 104 996
- US-A- 2 635 958

## Description

### Field of application

The present invention relates to a paper material comprising cellulose fibers and leather fibers. The invention also relates to a process for the production of the above-mentioned paper material.

### Known art

In the field of cellulose materials, in particular in the paper production industry, the problem of preserving the environment and reducing costs, is always relevant. For this reason considerable attention is paid to recycling techniques of paper materials, thus trying to limit the use of virgin cellulose material. The products obtained starting from recycled cellulose materials, however, have different physical properties from those obtained from virgin cellulose materials.

In the art, paper articles comprising both cellulosic and leather fibers are known from US 2104996 A, US 2635958 A and GB 2045829 A.

US1269905A discloses a process of making felt for roofing which consists in disintegrating scrap leather and cellulose fiber into a fibrous pulpy mass of the consistency of paper stock, adding a softening agent soft admixture of cellulose, adding bichromate of soda or potash to the pulp, and then forming the pulp into soft porous absorbent sheets.

US1211837A discloses a material composed of a highly absorbent flexible sheet comprising fibers of cotton or wool and leather felted together and saturated with a bituminous material.

The Applicant has considered the problem of providing a paper material having a fibrous component comprising alternative fibrous materials to virgin cellulose, preferably deriving from recycled materials, without jeopardizing the mechanical properties of the final paper product, such as, for example, rigidity, thickness, burst strength, rupture length. A further objective of the present invention is to provide this type of paper material which also has a high electric conductivity and high volume or "bulk" values.

The above objectives have been achieved by the Applicant through a paper material, wherein the cellulose fibers of the fibrous component are partially substituted by leather fibers, in particular leather fibers obtained from waste of the tanning industry and leather transformation.

### Summary of the invention

According to a first aspect, the present invention relates to a paper material wherein the fibrous component comprises leather fibers in a percentage within the range of 5-80% dry weight and cellulose fibers in a percentage within the range of 95-20% dry weight, wherein said dry weight percentages refer to the total dry weight of the fibrous component, and wherein said leather fibers and cellulose fibers form a homogenous mixture by means of a tanning agent.

The fibrous component of the paper material according to the invention preferably consists of cellulose fibers and leather fibers.

The paper material according to the present invention advantageously has a high electric conductivity and a high "bulk".

Another advantage relates to the fact that the use of leather fibers in substitution of cellulose fibers allows a considerably reduced quantity of virgin cellulose material, up to 80% less, to be used in the production of the paper material according to the invention.

A further advantage provided by the present invention is the possibility of effectively recycling the tanning industry and leather transformation residues.

Another advantage lies in the fact that the paper material of the invention is biodegradable or compostable, reducible to pulp and can therefore be recycled in the paper production chain.

Yet another advantage is represented by the fact that the paper material according to the present invention can be coupled with non-paper materials, in particular biodegradable plastic films such as PHA (polyhydroxyalcanoate), Mater-Bi^{®}, PLA (polylactic acid) to obtain compostable end-products, which can be used, for example, in the packaging industry.

For the purposes of the present invention, a material is considered "biodegradable" if it meets the biodegradability requirements established by the standard EN 13432.

For the purposes of the present invention, a material is considered "compostable" if it meets the compostability requirements established by the standard EN 13432.

For the purposes of the present description and enclosed claims, the verb "to comprise" and all terms deriving therefrom also include the meaning of the verb "to consist of" and all terms deriving therefrom.

The limits and numerical ranges expressed in the present description and enclosed claims also comprise the numerical value(s) mentioned. Furthermore, all the values and sub-ranges of a limit or numerical range should be considered as being specifically included as if explicitly mentioned.

Further features and advantages of the present invention will appear evident from the following detailed description.

### Detailed description

According to a preferred aspect of the present invention, the leather fibers have a length comprised within the range of 0.1-30 mm, preferably within the range of 1 - 20 mm, more preferably 4 - 15 mm.

Preferably, the leather fibers are obtained by the defibration of leather, more preferably leather obtained from wastes of the tanning industry and leather transformation industry, such as, for example, residues of shaving and splitting phases of tanning processes or trimming scraps of the leather transformation industry.

For the purposes of the present invention, the above-mentioned waste products are reduced to the state of fibers using processes and techniques known in the field of leather scrap recovery, in particular in the field of so-called "bonded leather" production.

In particular, the defibration can be obtained mechanically, by grinding the scraps in synchronized hammer and/or knife mills and/or defibration mills, preferably Pallmann defibration mills.

Preferably, the defibration process in mills is continued for a period of time that avoids the complete separation of the single fibers, but for a duration that is such as to obtain leather fibers in bundles, which is preferably a maximum of 30 minutes. It has in fact been observed that defibration times longer than those indicated above, damage the collagen fibers forming the leather, in addition to causing excessive energy consumptions.

The leather fibers are preferably partially defibrated.

The leather fibers are preferably in the form of bundles of fibers, more preferably similar to a tangle.

The fibers obtained from the defibration processes described above, have a morphology and dimensions similar to those of cellulose fibers. This makes the above leather fibers compatible with cellulose fibers, and they can therefore be used as part of the fibrous component of a paper material.

The use of leather fibers according to the present invention gives the paper material a characteristic aspect, as these fibers are at least partially visible also to the naked eye in the end-product, as pointed out in the enclosed figure 1 which shows a paper material according to the invention.

The presence of leather fibers in bundles can also be noticed in the enclosed figures 2 and 3 which show electron microscope images of a sample of leather fibers according to the invention. The presence of bundles of leather fibers offers the advantage of increasing the bulk value of the paper material obtainable, without substantially deteriorating the other properties.

The leather fibers are preferably obtained from leather tanned through tanning processes of the type that do not use chromium, more preferably vegetable tanning (for example, using tannin as tanning agent) or "wet white" tanning (e.g. using aldehydes as tanning agent). Vegetable and "wet white" tanning, in fact, do not use chromium. The use of fibers deriving from these tanned leathers in the production of paper material according to the present invention, therefore avoids all problems of an environmental nature relating to the use of this heavy metal.

The paper material of the present invention is preferably one or more selected from printing paper or cardboard; paper for the lining of boxes; paper for packaging; corrugated paper and cardboard; paper for shoppers and bags; paper for labels; and security paper.

The paper material is preferably coated, embossed, die-cut and/or laminated.

The paper material according to the present invention can be in various forms, for example in the form of a sheet having variable dimensions, in the form of a reel, etc.

According another preferred aspect, the paper material of the present invention has an electric conductivity within the range of 1×10⁻⁷ - 1×10⁻¹⁰ S/m, more preferably 1×10⁻⁸ - 1×10⁻⁹. This conductivity value makes the paper material according to the present invention particularly suitable for use as a support for digital printing, photostat printing and similar. For this kind of application, the fibrous component of the paper material preferably comprises leather fibers in a percentage within the range of 5 - 20%, more preferably 5 - 10% dry weight and cellulose fibers in a percentage within the range of 95 - 80%, more preferably 95 - 90% dry weight, wherein said dry weight percentages refer to the total dry weight of the fibrous component.

For comparative purposes, the typical electric conductivity of the paper produced with cellulose fibers alone is normally comprised within the range of 1×10⁻¹² - 1×10⁻¹⁴ S/m.

The paper material preferably has an absolute humidity within the range of 4-12%, more preferably 5-10%. The paper material preferably has a *bulk* value (thickness (um)/grammage (g/m²) ratio) within the range of 1.2-1.8, more preferably within the range of 1.4-1.7. These values are on an average about 25% higher than the bulk values obtainable for conventional paper materials, without leather fibers.

High bulk values are desirable for blotting paper, for example. Low bulk values are desirable for printing paper, for example. With the present invention a paper material can be obtained, having a desired bulk value, using a lower amount of cellulose fibers with respect to a conventional paper not containing leather fibers.

The paper material preferably has an organic nitrogen content within the range of 1-12%, more preferably 3-6% (Kjendahl method). This nitrogen content makes the paper material easily compostable.

The paper material preferably has a grammage within the range of 80-1,100 g/m², more preferably 100-600 g/m².

The paper material according to the present invention advantageously does not cause skin irritation. This evaluation can be effected by carrying out, for example, a patch test of the occlusive type.

The paper material according to the invention preferably has, on the surface, occlusions deriving from partially defibrated leather fibers. These occlusions give the material a characteristic or immediately recognizable appearance.

A second aspect of the present invention relates to a process for the production of a paper material as defined above and comprises the following steps:
a) preparing a water-based mixture comprising cellulose fibers and leather fibers, wherein the leather fibers are in a percentage comprised within the range of 5 - 80% dry weight and the cellulose fibers in a percentage within the range of 95 - 20% dry weight, wherein said dry weight percentages are based on the total dry weight of the sum of the cellulose fibers and the leather fibers;
   a-1) adding a tanning agent to the water-based mixture of said step a);
b) forming a layer of said mixture on a draining screen and draining the water contained in said mixture; and
c) drying said drained mixture so as to obtain said paper material.

In the present description and enclosed claims, the term tanning agent refers to a compound of the type generally used in the tanning processes of animal hides, that stabilizes the collagen.

For the purposes of the present invention, the addition of the tanning agent in step a) favours the formation of a homogeneous mixture of the leather fibers and cellulose fibers.

Preferably, the tanning agent is within the group which is selected from: mineral tanning agents (e.g. zirconium or aluminium salts), tannins, more preferably vegetable tannins, aldehydes (e.g. glutaraldehyde), tanning oils, or combinations thereof.

Preferably, the tanning agent is added in step a) in a dry weight percentage within the range of 0.1-2.0%, more preferably 0.2-0.8%, wherein said percentage refers to the total dry weight of the leather fiber.

One or more additives of the type commonly used in the paper industry, such as optical brightener agents, dyes, sizing agents, fillers (e.g. calcium carbonate and kaolin) silica, cationic starch, wet-strength agents, etc., are preferably added to the water-based mixture of step a), according to the characteristics desired for the final paper material.

Preferably, the dyes are present in a quantity within the range of 0.05 - 10.00% dry weight, wherein said percentage refers to the total dry weight of the mixture.

Preferably, step b) is preceded by a refining step of the mixture of step a), more preferably with the use of conical or disc refiners.

The process according to the present invention can be carried out with equipment known to skilled person in the paper industry field. Steps b) and c), in particular, can be effected with a continuous machine for the production of paper.

The paper material obtained at the end of step c) is preferably subjected to one or more finishing steps selected from the group comprising calendering, embossing, corrugation, coupling and coating.

In particular, the coating can be effected using techniques and equipment known to skilled person in the field, such as air knife coating, curtain coating, stiff blade, bent blade, metering and film press.

According to a third aspect, the present invention relates to the paper material obtained according to the above-mentioned production process.

According to a fourth aspect, the present invention relates to the use of the above-mentioned paper material for producing a biodegradable multilayer composite material together with one or more non-paper materials, in particular biodegradable plastic films, i.e. films comprising biodegradable polymers, such as cellulose acetate, PBS (polybutylenesuccinate), PHA (polyhydroxyalcanoate), Mater-Bi^{®}, PLA (polylactic acid), etc.

According to a fifth aspect, the present invention relates to a biodegradable multilayer composite material comprising at least one layer of the paper material described above, laminated with at least one biodegradable film.

Such composite material can be advantageously used for preparing biodegradable or compostable end-products, which can be used, for example, in the packaging and agricultural fields.

The biodegradable films that can be used for the purposes of the present invention are known to skilled persons in the field and can be found on the market. These films comprise biodegradable polymers such as, for example, polymers and copolymers of hydroxy acids (so-called poly(hydroxy acids)) - in particular polymers and copolymers of lactic acid and glycolic acid -, cellulose polymers, hydroxyalkanoate polymers (e.g. polyhydroxybutyrate-co-valerate (PHBV), biodegradable copolyesters (e.g. polybutylenesuccinate adipate (PBSA), polybutylene adipate-co-terephthalate), polycaprolactones (PCLs) and starch-based polymers.

The multilayer composite materials according to the present invention can be prepared by means of processes known to skilled persons in the field.

### Short description of the figures

Figure 1 shows a sample of paper material according to the invention;
Figure 2 is an electronic microscope image of a leather fiber sample according to the present invention;
Figure 3 is another electronic microscope image of a leather fiber sample according to the present invention;

### Examples

The present invention will now be further illustrated by means of some embodiment examples as described hereunder.

### Example 1: Paper material with 60% of leather fibers and 40% of cellulose fibers (cellulose soft wood NBSK).

### Composition 1:

- 300 kg of shaved leather tanned by means of the "wet white" technique (leather previously defibrated using a blade mill and for 10 minutes with a Pallmann defibrator mill);
- 300 kg of leather residues tanned by means of the "wet white" technique (residues previously chopped with a blade mill and defibrated for 20 minutes with a Pallmann defibrator mill);
- 400 kg of bleached chemical cellulose ASPA (NBSK);
- 20 kg of cold-soluble cationic starch;
- 50 kg of calcium carbonate;
- 20 kg of natural tanning agent, 50% of dry product (Chimotan OPS of Chimotan Group).

The materials of composition 1 were introduced into a vat and refined for 10 minutes, by means of conical refiners, in order to obtain the homogenization of the fibrous component. The mixture obtained, equal to 1,090 kg was added to a Fourdrinier continuous machine for the production of paper, with a production of 1,000 kg/h and a rate of 22 m/min, obtaining a reel of paper material. The final grammage of the paper material obtained was about 700 g/m², whereas the thickness was 1,100 microns. The final absolute humidity of the paper material was equal to 12%.

The paper material is biodegradable, recyclable and reducible to pulp. This latter feature makes the material suitable for further transformations of the paper process. Table 1 hereunder, item A, shows the characteristics of the paper material obtained.

### Example 2: paper material with 15% of leather fibers and optical bleacher for printing.

### Composition 2:

- 750 kg of paper material of example 1 cut into sheets;
- 2,000 kg of bleached chemical cellulose, of which: 500 kg of soft wood cellulose (NBSK) and 1,500 kg of hardwood cellulose (eucalyptus, beech, poplar, aspen);

- 200 kg of calcium carbonate;
- 25 kg of optical bleacher (Leucophor^{®} ACK of Archroma);
- 5 kg of natural tanning agent, 50% of dry product (Chimotan OPS of Chimotan Group).

The materials of composition 2 were dosed and the following products were added: cationic starch 15 kg dry, aluminium polychloride 30 kg as such, colloidal silica 4.5 kg dry and 30 kg of sizing agent based on AKD for the sizing of the paper. The latter materials are useful for retention.

The mixture was homogenized with a pulper, stored in a vat and dosed on a Fourdrinier continuous paper machine. The rate of the machine was 120 m/min, with an hourly production of 1,200 kg/h. A final smoothing was effected to make the paper suitable for printing. The final absolute humidity of the paper material was 7.0%. The production yield was equal to 2,700 kg as reels which were subsequently cut into sheets. The grammage of the paper was 120 g/m². During production, a solution of starch was applied to the surface by means of a size-press machine, in order to improve the surface characteristics of the paper and make it suitable for printing.

As resulting product, a paper material was obtained, that is recyclable, reducible to pulp, biodegradable, compostable and sized. The presence of the optical brightener agents makes the paper whiter, favouring its use as printing and writing paper. The presence of bundles of leather fibers gives the paper a characteristic appearance. Table 1 hereunder, item B, shows the characteristics of the paper material obtained.

### Example 3: paper material in reel of printing paper with 300 of leather fibers having a natural colour.

### Composition 3:

- 2,200 kg of the material obtained according to example 1 cut into sheets;
   - 2,000 kg of bleached chemical cellulose, of which: 500 kg of soft wood cellulose (NBSK) and 1,500 kg of hardwood cellulose (eucalyptus, beech, poplar, aspen);
   - 200 kg of calcium carbonate;
   - 10 kg of natural tanning agent, 50% of dry product (Chimotan OPS of Chimotan Group).

The following products were added to the materials of composition 3: cationic starch 15 kg dry, aluminium polychloride 30 kg as such, colloidal silica 4.5 kg dry, and 30 kg of size agent based on AKD for sizing the paper. These latter materials are useful for retention.

The mixture was homogenized with a pulper, stored in a vat and subsequently dosed on a Fourdrinier continuous paper machine. The rate of the machine was equal to 70 m/min, with an hourly production of 1,400 kg/h. The absolute humidity of the final paper material was equal to 7.5%. The production yield was equal to 4,200 kg. The paper grammage was 250 g/m². During the production, a starch solution was applied to the surface with a film-press machine in order to improve the surface characteristics of the paper, thus making the same suitable for printing. As resulting product, a paper material was obtained, which is recyclable, reducible to pulp, biodegradable, compostable and sized. The presence of bundles of leather fibers gives the paper a characteristic appearance.

Table 1 hereunder, item C, indicates the characteristics of the paper material obtained. Due to the presence of animal fibers, a test was carried out for assessing skin irritability (patch test of the occlusive type) which gave a negative result.

### Example 4: black paper material, with 300 of leather fibers, coloured with direct dyes.

### Composition 4:

- 2,200 kg of the paper material obtained according to example 1 cut into sheets;
- 2,000 kg of bleached chemical cellulose, of which: 500 kg of softwood cellulose (NBSK) and 1,500 kg of hardwood cellulose (eucalyptus, beech, poplar, aspen);
- 200 kg of calcium carbonate;
- 40 kg of Cartacrom 2T Black in powder form (CI: Direct Black 80);
- 40 kg of Cartacrom N Black in powder form (CI: Direct Black 168);
- 10 kg Cartacrom GTN Red 150% in powder form (CI: Direct Red 239).

The following products were added to the materials of composition 4: cationic starch 20 kg dry, aluminium polychloride 40 kg as such, colloidal silica 5.5 kg dry, and 30 kg of sizing agent on AKD for sizing the paper. These latter materials are useful for retention.

The mixture was homogenized with a pulper, stored in a vat for dyeing and then dosed on a Fourdrinier continuous paper machine. The rate of the machine was 120 m/min, with an hourly production of 1,200 kg/h in a reel. A final smoothing was effected to make the paper suitable for main paper transformations, in particular lamination. The final absolute humidity of the paper material was 7.0%. The production yield was equal to 4,250 kg. The paper grammage was 250 g/m². During production, a solution of starch and direct black dye was applied to the surface with a size-press machine, in order to improve the surface characteristics of the paper and increase the colour intensity of the paper.

As resulting product, a paper material was obtained, that is recyclable, reducible to pulp, biodegradable, compostable and sized, black in colour (L=26.5; a=0.7 b=-1.4) and characterized by whitish inclusions due to the presence of leather fibers that do not absorb direct dyes.

Table 1, item D, indicates the characteristics of the material obtained.

### Example 5: Coated paper with 300 of leather fibers.

A paper reel produced according to example 3, of 250 g/m² was coated with an air knife coating machine applying a coating equal to 10 g/m². The dry product of the coating was 35% and the pH was adjusted to a value of 8.5 with NaOH.

### Composition of the dry coating:

| | |
|---|---|
| polymethyl urea | 100 kg |
| precipitated calcium carbonate | 200 kg |
| kaolin | 100 kg |
| styrene-butadiene latex | 300 kg |
| Insolubilizing agents | 15 kg |
| Dispersing and wetting agents | 5 kg |
| Thickening agents | 6 kg |
| NaOH | 1 kg |
| Optical bleacher | 4 kg. |

As resulting product a paper material was obtained, which is recyclable, reducible to pulp, biodegradable, compostable, sized and coated, characterized by whitish inclusions due to the presence of collagen which absorbed the coating in a different way.

Table 1, item E, indicates the characteristics of the material obtained.

### Example 6: Embossing of the paper material according to the present invention

A paper reel produced according to example 2 (15% of leather fibers and optical brightener agents) of 120 g/m² was embossed with a UNIMATEC embosser at a rate of 100 m/min, a temperature of 75°C and a pressure of 80 bar. The steel marking cylinder was characterized by a width of 150 cm and a diameter of 25.34 cm. The absolute humidity of the final marked paper was 7.0%.

As resulting product, a paper material was obtained with a surface marking similar to canvas. The paper material thus obtained can be used for example in the coating of boxes.

### Example 7: biodegradable multilayer composite material

A paper reel produced according to example 3 (30% of leather fibers and a natural colour) of 250 g/m² was cut by means of a Jagemberg SYNCHRO cutter into a format of 72x102 cm and was coupled on a PAPERPLAST WD coupling machine with a cellulose acetate film ACE BLUE of CLARIFOIL of 32 g/m² using 4 g/m² of a biodegradable adhesive (aqueous dispersion based on polyester-polyurethane elastomers - EPOTAL P100 Eco of BASF). The absolute humidity of the final laminated paper was 7.0%, whereas the final grammage was 286 g/m².

As resulting product, a biodegradable multilayer composite material was obtained, which can be used for example in the production of compostable flower pots.

**TABLE 1: physico-mechanical characteristics of the paper materials obtained**

| | | | A | B | C | D | E |
|---|---|---|---|---|---|---|---|
| Type of paper | | | Ex. 1 | Ex. 2 | Ex. 3 | Ex. 4 | Ex. 5 |
| leather fibers | % | | 60 | 15 | 30 | 30 | 30 |
| grammage | g/m² | ISO 536 | 700 | 120 | 250 | 250 | 260 |
| Thickness | micron | ISO 534 | 1100 | 192 | 430 | 430 | 430 |
| bulk | | | 1.57 | 1.60 | 1.72 | 1.72 | 1.63 |
| L* | | | 77.8 | 88.9 | 80.2 | 26.5 | 82.0 |
| a* | | | 2.5 | 3.8 | 4.0 | 0.7 | 3.0 |
| b* | | | 16.5 | 1.8 | 18.7 | -1.4 | 12.0 |
| Bendtsen smoothness | ml/min | ISO 8791 | >2000 | 1000 | 1500 | 1300 | 800 |
| | | | >2000 | 900 | 1400 | 1000 | 1000 |
| Cobb 60s | g/m² | ISO 535 | 50 | 25 | 35 | 40 | 35 |
| Felt side | | | | | | | |
| Cobb 60s | g/m² | ISO 535 | 40 | 25 | 35 | 40 | 40 |
| Wire side | | | | | | | |
| Dennison waxes | N. | | 10/10 | 16/18 | 16/18 | 16-18 | 18-18 |
| Absolute humidity | % | | 12.0 | 7.0 | 7.5 | 7.0 | 7.0 |
| Occlusive Patch Test | | | | | Not irritating | | |
| Electric conductivity | S/m | | | 2x10⁻⁹ | 5x10⁻⁸ | 1x10⁻⁸ | |

## Claims

1. Paper material wherein the fibrous component comprises leather fibers in a percentage comprised within the range 5 - 80% dry weight and cellulose fibers in a percentage comprised in the range 95 - 20% dry weight, wherein said dry weight percentages are based on the total dry weight of the fibrous component, and wherein said leather fibers and cellulose fibers form a homogenous mixture by means of a tanning agent.

2. Paper material according to claim 1, wherein said leather fibers have a length comprised within the range 0.1 - 30 mm, preferably 1 - 20 mm, more preferably 4 - 15 mm.

3. Paper material according to claim 1 or 2, wherein the leather fibers are obtained through leather defibration, preferably leather obtained from scraps of the leather tanning and transformation industry.

4. Paper material according to any one of the preceding claims, wherein the leather fibers are obtained from leather tanned through tanning processes of the type that do not use chrome, preferably vegetal tanning or wet white tanning.

5. Paper material according to any one of the preceding claims, wherein said paper material has an electric conductivity in the range 1×10⁻⁷ - 1×10⁻¹⁰ S/m, more preferably 1×10⁻⁸ - 1×10⁻⁹ S/m.

6. Paper material according to any one of the preceding claims, wherein said material has an absolute humidity within the range 4 - 12%, preferably 5 - 10%.

7. Paper material according to any one of the preceding claims, wherein said material has a *bulk* value in the range 1.2 - 1.8, preferably in the range 1.4 - 1.7.

8. Paper material according to any one of the preceding claims having an organic nitrogen content comprised within the range 1 - 12%, preferably 3 - 6%.

9. Paper material according to any one of the preceding claims, having occlusions on the surface deriving from partially defibrated fibers.

10. Process for the manufacture of a paper material as defined in the preceding claims 1-9, comprising the steps of:
a) preparing a water-based mixture comprising cellulose fibers and leather fibers, wherein the leather fibers are present in a percentage comprised within the range 5 - 80% dry weight and the cellulose fibers in a percentage comprised within the range 95 - 20% dry weight, wherein said dry weight percentages are based on the total dry weight of the sum of the cellulose fibers and the leather fibers;
a-1) adding a tanning agent to the water-based mixture of said step a);
b) forming a layer of said mixture on a draining screen and draining the water contained in said mixture; and
c) drying said drained mixture so as to form said paper material.

11. Process according to claim 10, wherein said tanning agent is added to the water-based mixture of step a) in a dry weight percentage within the range 0.1 - 2.0%, preferably 0.2 - 0.8%, wherein said percentage is based on the total dry weight of the leather fibers.

12. Process according to any one of claims 10 or 11 wherein said step b) is preceded by a refining step of the mixture of step a), more preferably by using conical or disc refiners.

13. Process according to any one of claims 10 - 12 wherein, at the end of step c), said paper material is subjected to one or more refining steps selected from the group comprising calendering, embossing, corrugation, coupling and coating.

14. Use of the paper material according to any one of claims 1 - 9 for manufacturing a biodegradable multilayer composite material together with one or more non-paper materials, particularly biodegradable plastic films, such as PHA (polihydroxyalcanoates), materBi^{®}, PLA (polylactic acid).

15. A biodegradable multilayer composite material comprising at least one layer of a paper material according to claim 1 laminated with at least one biodegradable film.

## Patentansprüche

1. Papiermaterial, bei dem die Faserkomponente Lederfasern in einem Prozentsatz im Bereich von 5 bis 80% des Trockengewichts und Zellulosefasern in einem Prozentsatz im Bereich von 95 bis 20% des Trockengewichts umfasst, wobei die Trockengewichtsprozentsätze auf dem Gesamttrockengewicht der Faserkomponente basieren und wobei die Lederfasern und die Zellulosefasern mit Hilfe eines Gerbstoffs ein homogenes Gemisch bilden.

2. Papiermaterial nach Anspruch 1, wobei die Lederfasern eine Länge im Bereich von 0,1 bis 30 mm, vorzugsweise 1 bis 20 mm, besonders bevorzugt 4 bis 15 mm aufweisen.

3. Papiermaterial nach Anspruch 1 oder 2, wobei die Lederfasern durch Zerfaserung von Leder, vorzugsweise von Leder aus Abfällen der Ledergerberei und - verarbeitungsindustrie, gewonnen werden.

4. Papiermaterial nach einem der vorstehenden Ansprüche, wobei die Lederfasern aus Leder gewonnen werden, das durch Gerbverfahren des Typs gegerbt wurde, bei dem kein Chrom verwendet wird, vorzugsweise durch pflanzliche Gerbung oder nasse Weißgerbung.

5. Papiermaterial nach einem der vorstehenden Ansprüche, wobei das Papiermaterial eine elektrische Leitfähigkeit im Bereich von 1×10⁻⁷ bis 1×10⁻¹⁰ S/m, besonders bevorzugt 1×10⁻⁸ bis 1×10⁻⁹ S/m aufweist.

6. Papiermaterial nach einem der vorstehenden Ansprüche, wobei das Material eine absolute Feuchtigkeit im Bereich von 4 bis 12%, vorzugsweise 5 bis 10% aufweist.

7. Papiermaterial nach einem der vorstehenden Ansprüche, wobei das Material einen *Schüttwert* im Bereich von 1,2 bis 1,8, vorzugsweise im Bereich von 1,4 bis 1,7 aufweist.

8. Papiermaterial nach einem der vorstehenden Ansprüche mit einem Gehalt an organischem Stickstoff im Bereich von 1 bis 12%, vorzugsweise 3 bis 6%.

9. Papiermaterial nach einem der vorstehenden Ansprüche, mit Einschlüssen auf der Oberfläche, die von teilweise zerfaserten Fasern herrühren.

10. Verfahren zur Herstellung eines Papiermaterials gemäß den vorstehenden Ansprüchen 1 bis 9, umfassend die Schritte:
a) Herstellen eines Gemischs auf Wasserbasis, das Zellulosefasern und Lederfasern umfasst, wobei die Lederfasern in einem Prozentsatz im Bereich von 5 bis 80% des Trockengewichts und die Zellulosefasern in einem Prozentsatz im Bereich von 95 bis 20% des Trockengewichts vorhanden sind, wobei die Trockengewichtsprozentsätze auf dem Gesamttrockengewicht der Summe der Zellulosefasern und der Lederfasern basieren;
a-1) Zugeben eines Gerbstoffs zu dem Gemisch auf Wasserbasis aus Schritt a);
b) Bilden einer Schicht des Gemischs auf einem Abtropfsieb und Ablassen des in dem Gemisch enthaltenen Wassers; und
c) Trocknen des entwässerten Gemischs, um das Papiermaterial zu bilden.

11. Verfahren nach Anspruch 10, wobei der Gerbstoff dem Gemisch auf Wasserbasis aus Schritt a) in einem Trockengewichtsprozentsatz im Bereich von 0,1 bis 2,0%, vorzugsweise 0,2 bis 0,8% zugesetzt wird, wobei der Prozentsatz auf dem Gesamttrockengewicht der Lederfasern basiert.

12. Verfahren nach einem der Ansprüche 10 oder 11, wobei dem Schritt b) ein Veredelungsschritt des Gemischs aus Schritt a) vorausgeht, vorzugsweise unter Verwendung von Kegel- oder Scheibenrefinern.

13. Verfahren nach einem der Ansprüche 10 bis 12, bei dem am Ende von Schritt c) das Papiermaterial einem oder mehreren Veredelungsschritten unterzogen wird, ausgewählt aus der Gruppe bestehend aus Kalandrieren, Prägen, Riffeln, Koppeln und Beschichten.

14. Verwendung des Papiermaterials nach einem der Ansprüche 1 bis 9 zur Herstellung eines biologisch abbaubaren Mehrschicht-Verbundmaterials zusammen mit einem oder mehreren Nicht-Papiermaterialien, insbesondere biologisch abbaubaren Kunststofffolien, wie PHA (Polyhydroxyalkanoate), materBi^{®}, PLA (Polymilchsäure).

15. Biologisch abbaubares Mehrschicht-Verbundmaterial, umfassend mindestens eine Schicht aus einem Papiermaterial nach Anspruch 1, die mit mindestens einer biologisch abbaubaren Folie laminiert ist.

## Revendications

1. Matériau de papier dans lequel le composant fibreux comprend des fibres de cuir dans un pourcentage compris entre 5 et 80% en poids sec et des fibres de cellulose dans un pourcentage compris entre 95 et 20% en poids sec, dans lequel lesdits pourcentages en poids sec sont basés sur le poids sec total du composant fibreux, et dans lequel lesdites fibres de cuir et lesdites fibres de cellulose forment un mélange homogène au moyen d'un agent tannant.

2. Matériau de papier selon la revendication 1, dans lequel lesdites fibres de cuir ont une longueur comprise entre 0,1 et 30 mm, de préférence entre 1 et 20 mm, de manière davantage préférée entre 4 et 15 mm.

3. Matériau de papier selon la revendication 1 ou 2, dans lequel les fibres de cuir sont obtenues par défibrage du cuir, de préférence du cuir obtenu à partir de déchets de l'industrie du tannage et de la transformation du cuir.

4. Matériau de papier selon l'une quelconque des revendications précédentes, dans lequel les fibres de cuir sont obtenues à partir de cuir tanné par des procédés de tannage n'utilisant pas de chrome, de préférence un tannage végétal ou un tannage blanc humide.

5. Matériau de papier selon l'une quelconque des revendications précédentes, dans lequel ledit matériau de papier a une conductivité électrique comprise entre 1×10⁻⁷ et 1×10⁻¹⁰ S/m, de manière davantage préférée entre 1×10⁻⁸ et 1×10⁻⁹ S/m.

6. Matériau de papier selon l'une quelconque des revendications précédentes, dans lequel ledit matériau présente une humidité absolue comprise entre 4 et 12%, de préférence entre 5 et 10%.

7. Matériau de papier selon l'une quelconque des revendications précédentes, dans lequel ledit matériau a une valeur *en gros* comprise entre 1,2 et 1,8, de préférence entre 1,4 et 1,7.

8. Matériau de papier selon l'une quelconque des revendications précédentes, ayant une teneur en azote organique comprise entre 1 et 12%, de préférence entre 3 et 6%.

9. Matériau de papier selon l'une quelconque des revendications précédentes, présentant des occlusions à la surface provenant de fibres partiellement défibrées.

10. Procédé de fabrication d'un matériau de papier tel que défini dans les revendications précédentes 1 à 9, comprenant les étapes suivantes:
a) la préparation d'un mélange à base d'eau comprenant des fibres de cellulose et des fibres de cuir, dans lequel les fibres de cuir sont présentes dans un pourcentage compris entre 5 et 80% en poids sec et les fibres de cellulose dans un pourcentage compris entre 95 et 20% en poids sec, dans lequel lesdits pourcentages en poids sec sont basés sur le poids sec total de la somme des fibres de cellulose et des fibres de cuir;
a-1) l'ajout d'un agent tannant au mélange à base d'eau de ladite étape a);
b) la formation d'une couche dudit mélange sur une grille d'égouttage et l'égouttage de l'eau contenue dans ledit mélange; et
c) le séchage dudit mélange égoutté de manière à former ledit matériau de papier.

11. Procédé selon la revendication 10, dans lequel ledit agent tannant est ajouté au mélange à base d'eau de l'étape a) dans un pourcentage de poids sec compris entre 0,1 et 2,0%, de préférence entre 0,2 et 0,8%, dans lequel ledit pourcentage est basé sur le poids sec total des fibres de cuir.

12. Procédé selon l'une quelconque des revendications 10 ou 11 dans lequel ladite étape b) est précédée d'une étape de raffinage du mélange de l'étape a), de manière davantage préférée en utilisant des raffineurs coniques ou à disque.

13. Procédé selon l'une quelconque des revendications 10 à 12 dans lequel, à la fin de l'étape c), ledit matériau de papier est soumis à une ou plusieurs étapes de raffinage choisies dans le groupe comprenant le calandrage, le gaufrage, l'ondulation, le couplage et le revêtement.

14. Utilisation du matériau de papier selon l'une quelconque des revendications 1 à 9 pour la fabrication d'un matériau composite multicouche biodégradable avec un ou plusieurs matériaux non papier, en particulier des films plastiques biodégradables, tels que les PHA (polyhydroxyalcanoates), le materBi^{®}, le PLA (acide polylactique).

15. Matériau composite multicouche biodégradable comprenant au moins une couche d'un matériau de papier selon la revendication 1, stratifié avec au moins un film biodégradable.
